

June 19, 1956

C. F. GEESE

2,750,881

LITHOGRAPHIC PLATE PROCESS

Filed Aug. 15, 1952



INVENTOR  
Charles F. Geese  
BY  
Curtis, Morris & Safford  
ATTORNEYS

1

2,750,881

## LITHOGRAPHIC PLATE PROCESS

Charles F. Geese, Old Greenwich, Greenwich, Conn., assignor to Steel Dot Corporation, Old Greenwich, Conn., a corporation of Connecticut

Application August 15, 1952, Serial No. 304,484

1 Claim. (Cl. 101—149.2)

This invention relates to chromium plated metal plates, particularly plates which are useful in lithography, to methods of making such plates, to lithographic plates, and to the art of lithography.

In lithographic printing a lithographic plate which may be either stone or metal has a printing image reproduced on its surface so that an oil base ink preferentially adheres to the image, and moisture preferentially adheres to the intervening surfaces. For example, treated aluminum plates or treated zinc plates have been employed for such printing. Also, plates with plated coatings such as chrome plated copper on zinc, copper on stainless steel, and chrome on copper on steel have been used. These known plates not only are relatively expensive but are capable of printing only a limited number of impressions, for example, of the order of one or two hundred thousand impressions per plate.

It is an object of the present invention to overcome the difficulties and disadvantages of prior lithographic plates and methods of manufacture and to provide plates which are made of inexpensive materials, which have excellent printing characteristics, which resist wear and corrosive deterioration, which may be manufactured without difficulty and, importantly which are capable of making several million printing impressions. Other objects and advantages of the invention will be made apparent by the following description.

In one of its broader aspects the invention may be said to lie in providing a lithographic plate wherein the image is produced in fine grainy steel (such as low carbon steel of the low SAE 1000 series) and wherein the non-printing or open surfaces are covered with passivated chromium which is substantially non-porous and will not accept ink and retains sufficient moisture to repel grease and ink. In another aspect the invention may be said to lie in a chromium plated steel lithographic plate wherein exposed steel or image portion thereof has been so treated that a highly tenacious bond or attraction exists between the rubbed-in ink and the steel image. In still another aspect of the invention, it may be said to lie in providing a substantially non-porous chromium plating over ordinary steel or iron without the interposition of another plating material and in a relatively rapid manner by high current density.

The features of the invention may perhaps best be appreciated by reference to the accompanying drawing, and subsequent description wherein:

Figure 1 is a diagrammatic, simplified view of an offset printing press showing the relative positioning of the plate roll, the rubber blanket roll and the impression roll.

Figure 2 is a fragmentary cross-sectional view of a low carbon steel plate.

Figure 3 a cross-sectional view of the steel plate shown in Figure 1 after it has been chrome plated according to the invention.

Figure 4 is a cross-sectional view of the plate of Figure 3 after a light sensitive bichromate gel coating has been placed over the chrome plate.

2

Figure 5 is a view of the plate of Figure 4 and illustrates diagrammatically the existence of light-hardened areas on the gel and soft gel areas after a photographic image has been developed on the gel.

Figure 6 is a view of the same plate after it has been etched so that the image is reproduced in steel, the overlying chrome plate in such areas having been dissolved away by the etching solution.

Figure 7 is a view of the plate shown in Figure 6 after the gel coating has been washed off, exposing the steel printing surfaces and the chrome-plated non-printing surfaces.

Figure 8 is a diagrammatic view of the plate of Figure 7 which illustrates the activation of the steel printing surfaces and the passivation of the chrome or water-wettable surfaces.

Referring more particularly to Figure 1, the offset printing press 11 is shown as comprised of plate press roll 12 which receives ink from fount 13 by means of transfer rolls 14 and water from fount 15 by transfer rolls 16. Rubber blanket roll 17 picks up the ink impression from press roll 12. Paper 19, carried by rollers 20 passes between blanket roll 17 and impression roll 18, thereby receiving the printing impressions.

Now referring more particularly to Figures 2-8 which show the plates, the low carbon steel plate 21 of Figure 2 is first scrubbed thoroughly with a weak solution of phosphoric acid and pumice to clean it, or given a pickling treatment, and finally washed with water. Thereupon, the cleaned plate 21 is immersed in a chromium plating bath (not shown) which is of standard composition. For example, the plating bath may contain about 30 to 50 ounces of chromic acid per gallon and about 0.3 to 0.5 ounce of sulfuric acid per gallon so that the chromate-sulfate ratio is about 100:1. Some 6 to 8 volts are applied and a current density of approximately 1½ amperes per square inch of steel is maintained. The plating bath is held at a temperature of about 105° to 110° F. and plating continued for about 3 to 4 minutes. These conditions yield directly on the steel a highly adhesive chrome plate 22 which is relatively non-porous and which is about 0.00005 inch thick. It is to be understood that variations in the plating conditions may be made within the spirit of the invention. For example, one may chrome plate steel plates which have previously been polished or inspected to insure that holes and other surface defects are absent. Additionally, one may conduct the chrome plating step as a substantially continuous operation where the steel plate is introduced to the plating bath as a long strip thereafter being cut into the desired sizes.

Plate 21 with its chrome coating 22 is next coated with a thin layer of light-hardenable gum or gelatine, e. g., potassium bichromate gum, and dried as in the preparation of known lithographer's plates. Next, the gum coated plate 21 is exposed and developed by placing over the light sensitive gum coating 23 a photographic film which bears the non-transparent half-tone image to be imprinted. Plate 21 and the film (not shown) are placed in a vacuum holder under a strong light such as a mercury arc so that the parts 23a of gum coating 23 in register with the light transparent parts of the film are light hardened. The plate 21 is removed from the holder and the unhardened areas of gum coating 23 washed away by warm water. The image areas 24 of plate 21 which were under the soft gum sections are then etched with a standard etching solution for chrome plate, e. g. hydrochloric acid or calcium chloride mixtures, to remove the exposed chrome plate and yield the desired image etched to expose the grainy steel surface.

Upon completion of the etching step, the plate is next washed free of the remaining gum or gelatine which protected the non-printing chrome surfaces 23, by immers-

ing the plate in a hot alkali-type detergent solution which advantageously contains synthetic organic detergents such as organic-sodium wetting agents. I have had good results using either Oakite #27, a proprietary product presently available from Oakite Products, Inc., of New York, New York, and which is believed to be a heavy duty alkaline type metal cleaner. After the detergent wash, the etched plate is rinsed with water, and traces of oxidation on the front of the plate removed with a weak solution of orthophosphoric acid which not only cleans steel surfaces 24 but also renders chrome plate surfaces 23 "passive" and leaves it in a condition to accept a moisture film, whereby to make it repellent to oily or greasy substances such as ink.

Next the exposed steel surfaces 24 are to be rendered permanently ink receptive. I accomplish this by applying with soft rags a blueing solution which attacks the steel only. A representative formulation of this solution is made by mixing:

*Formula A*

|                    | Oz. |
|--------------------|-----|
| Bismuth chloride   | 1   |
| Sodium hyposulfite | 2   |
| Copper chloride    | 1   |
| Hydrochloric acid  | 6   |
| Alcohol (ethyl)    | 5   |
| Water              | 64  |

to yield a solution which in turn is mixed with, in equal parts, a hydrocarbon base liquid detergent. I use liquid detergents which have a hydrocarbon base and contain small amounts of wetting agents and soaps. Particularly good results have been achieved with a mixture of equal parts of kerosene and the liquid detergent known as Oakite #96, which is also available from Oakite Products, Inc., and which is an emulsion type cleaner comprised of various wetting agents with organic and hydrocarbon materials.

In place of Formula A other equivalent solutions or mixes which blacken steel may be used so long as they do not contain such an excessive proportion of hydrogen sulfide forming components as to be deemed objectionable as health hazards. Next, I wash off the steel blueing-detergent mixture with water and, while the odor of hydrogen sulfide is still detectable on the plate, I activate the blackened steel surfaces 24 with a dilute (e. g. 15%) solution of orthophosphoric acid by spreading on the solution with a cloth.

After activation and while the plate is still wet I apply a standard rub-in ink to the steel image thereby forming a very tenacious bond between the steel and the ink. The moisture on the chrome surfaces tends to repel the ink, and the ink is thus preferentially applied to the activated steel portions of the plate. If the plate is not to be used immediately, a gum arabic or similar protective coating is

preferably applied to the treated plate to protect it until needed in service.

By my invention there are produced lithographic plates which are inexpensive, strongly resistant to abrasion and wear of the non-printing or chrome plated surfaces and which are permanently ink receptive in the activated steel areas. Additionally, the tenacious ink to steel bond protects the steel printing surfaces from oxidation and corrosion.

Although in the foregoing specification I have given various examples of my invention and have suggested certain modifications and alternatives, these are not intended to be exhaustive of my invention but on the contrary are selected and presented with a view to illustrating and explaining the invention, the principles thereof and the best manner of applying it in practical use in order that others skilled in the art may be enabled to practice the invention and apply it under various circumstances and in various ways, and with modifications, each as may be best suited to the conditions of a particular use.

I claim:

In the process of making a chrome-on-steel lithographic plate whereon an image has been etched on steel, the steps of passivating chrome plated areas of the plate with dilute phosphoric acid, then rendering the etched steel portions of the plate ink receptive by treating said plate with a water-oil-detergent-acidic-metallic chemical blueing solution which evolves hydrogen sulfide on contact with steel, said blueing solution comprising (a) about one part of a mixture of equal parts of kerosene and a hydrocarbon base liquid detergent, and (b) about one part of a solution comprised of approximately 64 ounces of water, 5 ounces of alcohol, 6 ounces of hydrochloric acid, 1 ounce of copper chloride, 2 ounces of sodium hyposulfite and 1 ounce of bismuth chloride, next treating the plate with a dilute solution of phosphoric acid, and then applying rub-in ink to the plate while the plate is still moist.

**References Cited in the file of this patent**

**UNITED STATES PATENTS**

|           |              |               |
|-----------|--------------|---------------|
| 773,368   | Bower et al. | Oct. 25, 1904 |
| 951,103   | Cornwall     | Mar. 8, 1910  |
| 2,042,003 | Huebner      | May 26, 1936  |
| 2,203,849 | Trist        | June 11, 1940 |
| 2,289,443 | Mange        | July 14, 1942 |
| 2,302,669 | Batcheller   | Nov. 24, 1942 |
| 2,519,672 | Lawless      | Aug. 22, 1950 |
| 2,527,232 | Scroxton     | Oct. 24, 1950 |

**FOREIGN PATENTS**

|        |               |               |
|--------|---------------|---------------|
| 29,507 | Great Britain | June 16, 1910 |
|--------|---------------|---------------|

**OTHER REFERENCES**

Modern Electroplating. Special volume, 2d ptg., August 1942. The Electrochemical Society, N. Y. Only pp. 119 and 122 cited. (Copy available in Div. 56.)